

# UNITED STATES PATENT OFFICE.

FREDERIC EUGENE IVES, OF PHILADELPHIA, PENNSYLVANIA.

COLOR PHOTOGRAPH OR FILM AND METHOD OF PRODUCING SAME.

1,376,940.

Specification of Letters Patent.

Patented May 3, 1921.

No Drawing.

Application filed September 26, 1919. Serial No. 326,536.

To all whom it may concern:

Be it known that I, FREDERIC EUGENE IVES, a citizen of the United States, residing at Philadelphia, in the county of Philadelphia and State of Pennsylvania, have invented certain new and useful Improvements in Color Photographs or Films and Methods of Producing Same, of which the following is a specification, reference being 10 had therein to the accompanying drawing.

This invention is a novel color photograph or film and method of producing same. The invention involves both the arts of color photography and motion pictures, 15 and constitutes an improvement in both arts. The invention relates more particularly to a system of color photography or color motion pictures in which only two, instead of the theoretically necessary three, 20 color selection negatives are produced, from which two color positives are subsequently produced and suitably blended for exhibiting or projecting. The two-image plan has been heretofore tried, but the results have 25 been too inaccurate to be wholly satisfactory. The attempt to obtain the more perfect effects of a three-image system by means of two images is at best a compromise, but the systems heretofore tried have been 30 quite defective in color rendering, and it is the main object of the present invention to afford in a two-image system a better compromise, that is, a better representation of the colors of nature which the three-image 35 system would afford. Further objects and advantages of the present invention will be pointed out in the hereinafter following description of one embodiment hereof, or will be apparent to those skilled in the art.

Before describing the present invention, it will be advantageous to refer in outline to prior known systems. In the three-image system three negatives are made, namely, by selective exposure to red light, to green light, and to blue-violet, which will be termed blue light. These are the primaries. From such negatives secondaries of the respective complementary colors, namely, blue-green, magenta-pink and yellow are 50 produced and blended. With the two-image system heretofore tried the R negative, representing the red rays, has been produced as before, and the G negative, representing the green rays, but the B negative has been 55 simply omitted, followed by the omission of the yellow secondary or positive element in

the final picture. A positive of blue-green or preferably green has been produced from the R negative, and a positive of some selected red from the G negative, and these 60 blended to secure an approximation of the original. With such system no yellows are reproduced, these appearing white, a distinct defect. If a green positive from the R negative has been produced, no blues or 65 blue-greens are possible. If blue-green or peacock blue is the selected positive color, no true greens are producible. Orange colors appear as dilute red, and various other important hues are objectionably falsified. 70

The general plan of the present improvement is, instead of employing the usual R positive of a green or blue, and the usual G positive of a red secondary color, to substitute for one of these a dichroic image 75 showing the deeper secondary color at the thicker or denser parts of the image, and yellow at the thinner or more transparent parts. Thus, if the blue-green R positive is replaced by a dichroic image, the latter 80 may be described as a dichroic yellow-to-blue-green image. I prefer, however, and find it more practical to replace the usual G positive, that is, the red image, by a dichroic image which may be termed a dichroic yellow-to-red image; and I will 85 herein describe how to produce such a dichroic image, giving yellow in the palest portions, orange in the intermediate and red in the deepest portions of the image. I 90 will first describe the result of such composite or two-image color photograph or motion picture film.

In the first place, in carrying out the present novel system I prefer from the R 95 negative to produce an R positive of a blue-green color, although, as is well known, the shade may be varied to any point between blue and green. In exposing for the other or G negative I prefer to admit to the sensitive film a slight amount of blue light, enough to give a pale or feeble effect. From this a positive dichroic yellow-to-red image is produced, as already stated. The result will be that, when this image is blended with 100 the blue-green image, desirable colors and shades are possible in the final picture which render it far more practical and pleasing, as compared with prior systems. I will now 105 describe the result of this present system 110 with regard to certain specific colors.

Taking yellow light in the subject to be

photographed, this will simply develop white or clear in the first or R positive; yellow light passes freely through to the R sensitive plate. In the second or G image, 5 owing to the admission of a trace of blue in addition to green rays, yellow (minus-blue) will be represented and will reproduce palely, with the result that yellow in the subject is represented by the lightest or thinnest shades or parts of the dichroic or positive image. Thus, yellow is afforded in the final or blended picture. The fact of having yellow so represented enables the first positive image to be of a true peacock blue, so 10 that peacock blue hues are reproduced without degradation.

A true green, fully differentiated from the peacock shade, is producible as follows. Light of this color in the subject is shut out 20 in exposing for the R negative, with the result of yielding a dark or deep blue-green positive. In the other positive this color would under the prior system appear as white, but owing to the admission of a slight amount of blue light with the green, the 25 result is that the color is palely represented in the dichroic positive. That is, it reproduces as a yellow. This yellow, blended with the blue-green of the first positive 30 image, reduces the latter to a true green color.

Red light, of course, gives clear or white in the first positive image, but full and deep shades in the second. This being a dichroic 35 image which is red in the deeper shades, we have satisfactory reproduction of the reds. The oranges similarly affect the images, except that the depth is medium instead of full, and the dichroic image is orange-colored in its medium portions.

Pure white light gives an absolutely clear or white positive image from both negatives, and therefore white is reproduced.

Thus, all the main colors are desirably 45 represented in the final blended image. This is not claimed to be as perfect as a three-image picture, but, on the other hand, the limitations are more obvious from a scientific than from a practical or pictorial aspect. Cobalt blue will appear almost black, and pinks and purples will appear dull and reddish, but, as stated, the main primary and secondary colors which are of the greatest 50 importance are reproduced sufficiently accurately for pictorial purposes. Thus, for portraiture flesh color reproduces well, and also blue, gray and brown for the eye, and yellow, auburn and brown for the hair. With landscapes the green foliage and blue 55 skies are properly differentiated, and fruits and flowers will reproduce in yellows, oranges and reds.

I will now explain the dichroic or yellow-to-red image above referred to. Dichroism 60 is the property of a substance of appearing

in different colors under different conditions. For example, the organic substance chlorophyl, if examined in solutions of considerable thickness, appears red, but in thin layers appears green; it is dichroic. There 70 are certain dyes or dye combinations that exhibit the same properties. For example, an almost saturated solution of auramin, a yellow dye, to which has been added a small quantity of saffranin, a red dye, appears 75 yellow in thin layers, orange in medium layers and red in the thickest layers. This is not the equivalent, but is the contrary, of the employment of an ordinary red dye which has been heretofore proposed, the latter 80 not being dichroic, and in its thinner layers appearing as pale red, and in its thicker layers as deep red.

From the above it is thought it will be understood by those skilled in the art how 85 to produce the dichroic image and to blend it with the other selectively produced image. I will, however, refer to certain available methods. Thus, the imbibition method referred to in my prior Patents Nos. 1,121, 90 187, of December 15, 1914, and 1,186,000, of June 6, 1916, is available. From the second or G negative exposed by green light with a slight amount of blue is produced a gelatin relief positive in accordance with the prior 95 patents. This may first be thoroughly dyed in a solution of red or magenta dye stuff, and then transferred to a yellow dye bath for a moderate length of time, when it will be found that the yellow has substantially 100 displaced the red in the thinnest layers of the image. The result is the desired dichroic yellow-to-red positive image. Suitable formulæ may be as follows.

For the red dye:

|                                                                                |                |
|--------------------------------------------------------------------------------|----------------|
| Fast red D (sodium salt of p-sulfonaphthalene-azo-B-naphthol-di-sulfonic acid) | 1½ grams       |
| Acetic acid                                                                    | 5 c. c.        |
| Water                                                                          | 1000 c. c. 110 |

For the yellow dye:

|                                                                     |            |
|---------------------------------------------------------------------|------------|
| Brilliant yellow (sodium salt of disulfo-stilbene-disazo-bi-phenol) | ½ gram 115 |
| Acetic acid                                                         | 5 c. c.    |
| Water                                                               | 1000 c. c. |

Simultaneous rather than such successive dyeing may be employed. For example, a 120 mixture of a very soluble acid red or magenta dye having but slight affinity for gelatin, with a so-called direct yellow dye, having great affinity for gelatin will give the desired result. The relief print immersed in such 125 solution will be found to first dye red, which is later partly replaced by yellow, this action taking place earlier and more completely in the thinnest layers, giving again the yellow-to-red dichroic image. The dyes set 130

forth above will act in this manner when mixed together in proper proportions. Such a relief image may be blended with a blue-green image from the other negative in various ways. According to the patents mentioned it will be brought physically into contact with the final print or carrier, so that while moist the dichroic image will be transferred by imbibition and thus blended with the blue-green image already or later formed. This method is good for affording final color prints on paper. Another is to bodily superpose the relief print with a separately formed blue-green print, as described in my Patent No. 1,122,935, of December 29, 1914.

For motion pictures I prefer the mordant dye method of creating the dichroic image. Suitable dyes may be mordanted by proper metallic mordants. For example, a silver positive image may be produced from the G negative. This, when dry, may be immersed in a solution made up of water, 1000 c. c., potassium ferricyanid, 5 grams, chromic acid, 5 grams. This converts the silver into a transparent image, composed of silver ferricyanid. After thorough washing this image will take up basic dyes. For example, red may be first applied, and later yellow to replace the red in the paler shades. Saffranin red and auramin yellow dyes are suitable. The resulting dichroic image may be blended with a peacock blue image from the R negative by resensitizing the colloid layer with ferric ammonium citrate and printing a cyanotype image in the same layer similarly to my prior Patent No. 1,278,668, of September 10, 1918. If desired the peacock blue image may be produced as a separate print and superposed upon the dichroic yellow-to-red print.

Equivalent results are obtainable by producing three positive images from the two negatives. From the first negative I may make the usual positive. From the second negative I may make a first positive, under-exposed and contrasty, and produce this in a magenta or red color, and from the same negative a second positive fully exposed and soft, to be colored yellow. Suitable blending of these with each other and with the first positive will give approximately the results sought.

It will thus be seen that I have described a color photograph or film and method of producing the same, embodying the principles and attaining the advantages of the present invention. Since many matters of relative detail, such as the particular steps or order of steps employed, and the ingredients or formulæ used may be variously modified without departing from the underlying principles, it is not intended to limit the

invention to such features except in so far as specified in the appended claims. 65

What is claimed is:

1. The method of producing a color photograph or motion picture film by two blended or blendable images consisting in producing a dichroic image showing two secondaries and blending it with a second image showing the third secondary. 70

2. The method of producing a color photograph or motion picture film from two color selection negatives consisting in producing 75 positive images from one negative showing in two secondary colors and from the other negative showing in the third secondary.

3. The method of producing a color photograph or motion picture film from two color 80 selection negatives consisting in producing a dichroic positive image from one negative showing yellow in the thin places and another secondary color in the deep places and blending the same with a positive from the 85 other negative showing the third secondary color.

4. The method of claim 3, and wherein the first negative is exposed mainly to green and slightly to blue light and from which is 90 produced a yellow-to-red dichroic positive, blended with a blue-to-green positive from the other negative.

5. The method of claim 1, and wherein the dichroic image is produced by selective 95 dyeing of colloid material by two dyes acting differently upon the colloid.

6. The method of claim 1, and wherein the dichroic image in colloid is produced by successive dyeing in dyestuffs of different 100 colors and actions.

7. Method of producing a yellow-to-red dichroic image in a selectively absorbent gelatin layer consisting in dyeing in a red dye and then transferring to a yellow dye 105 until the red is displaced in the thin places.

8. A color photograph or motion picture film having two blended photographic images, one of which is dichroic to show two secondary colors, the other showing the 110 third secondary.

9. A color photograph or motion picture film having two blended photographic images, one of which is a yellow-to-red dichroic image, the other a blue-green image. 115

10. A support or base carrying a dichroic image for color photography wherein the thin parts show distinct colors from the deeply colored parts.

11. A support or base carrying a dichroic 120 image showing yellow in the thin places, orange in the deeper and red in the deepest.

In testimony whereof, I have affixed my signature hereto.

FREDERIC EUGENE IVES.